

## UNITED STATES PATENT OFFICE

2,228,507

## SOLVENT REFINING OF HYDROCARBON OIL

Leon W. Cook, Beacon, N. Y., assignor to The Texas Company, New York, N. Y., a corporation of Delaware

No Drawing. Application June 13, 1937,  
Serial No. 148,954

1 Claim. (Cl. 196—13)

This invention relates to refining hydrocarbon oil, and particularly to the solvent refining of residual lubricating oil fractions derived from petroleum.

5 The invention contemplates extracting hydrocarbon oil with furfural in the presence of chlorphenol. It has particular reference to extracting residual lubricating oil stock with these two solvents, whereby a lubricating oil product is produced having characteristics superior to those of a product obtained by extracting with the individual solvents alone. The product so obtained, for example, has a high viscosity index, coupled with a low residual carbon content.

15 Moreover, a higher yield of such oil can be obtained from the same stock by treating it in accordance with the method of this invention.

More specifically, the invention comprises extracting residual lubricating oil stock with furfural and chlorphenol, such as parachlorphenol, or a mixture of para and orthochlorphenol comprising around 60 to 70% of the para compound.

I have discovered that the addition of parachlorphenol, or a chlorphenol mixture consisting mainly of the para isomer, very greatly improves the effectiveness of furfural as an extraction solvent for residual lubricating oil stocks, particularly from the standpoint of producing a refined oil of low residual carbon content and of improved color.

Parachlorphenol exerts a comparatively high degree of solvent action upon the asphaltic and dark-colored constituents of residual oils. At the same time, it also exerts selective action as between low and high viscosity index constituents of the oil, although in this respect, it is less selective than furfural, and particularly if the parachlorphenol has associated with it substantial amounts of the orthochlorphenol. The orthochlorphenol is substantially completely miscible with lubricating oil in all proportions at all temperatures above its solid point. Consequently, the ortho compound fails to exert selective action as between low and high viscosity index constituents of the oil. Its presence, therefore, impairs the selective action of the para compound, especially if present in large amount.

However, by the procedure of my invention, the 50 lack of selective action possessed by the ortho constituent of the chlorphenol mixture is offset by the highly selective action of furfural. The furfural thus acts as an anti-solvent for the high viscosity index or paraffinic constituents of the 55 oil.

My invention, therefore, combines a high degree of selective action as between low and high viscosity index constituents of residual oil with a high degree of solvent action upon the residual carbon-forming and dark-colored constituents of the oil. 5

As a result, by employing the solvent mixture of my invention, it is possible to obtain a raffinate or refined oil from residual lubricating oil fractions which are of high viscosity index, low 10 in residual carbon content and of relatively good color. The product thus obtained since it combines these characteristics is superior to that obtained by employing either furfural or chlorphenol alone. 15

Reference will now be made to the following tables comprising data obtained by extracting a residual lubricating oil fraction derived from Mid-Continent crude with:

- (1) Furfural alone,  
(2) Parachlorphenol alone, and  
(3) A mixture of equal parts of furfural and parachlorphenol.

Table I shows the relationship between residual 25 carbon content and yield of raffinate when extracting with the three solvents:

TABLE I  
Carbon residue\* content—Per cent by weight of 30 raffinate

| Raffinate, percent by volume | Solvent         |                             |                                              | 35 |
|------------------------------|-----------------|-----------------------------|----------------------------------------------|----|
|                              | Furfural<br>(1) | Parachlor-<br>phenol<br>(2) | Furfural<br>plus para-<br>chlorphenol<br>(3) |    |
| 55                           | 5.4             | 2.25                        | 2.6                                          |    |
| 65                           | 5.5             | 3.2                         | 3.5                                          | 40 |
| 70                           | 5.6             | 3.6                         | 4.0                                          |    |
| 80                           | 6.0             | 4.6                         | 4.7                                          |    |

\*Conradson carbon.

The lubricating oil residuum had a residual carbon content of about 6.7% and, as indicated by the foregoing table, the raffinate obtained by extracting with furfural still had a high residual carbon content, ranging from 5.4 to 6.0%. Where the raffinate amounted to 55% of the residuum the residual carbon content was 5.4%, while in the case of a raffinate amounting to 80% of the residuum, the residual carbon content was 6.0%. 45

In contrast, when extracting with parachlor-

55

phenol alone, obtaining the same yields of raffinate, the residual carbon content ranged from 2.25 to 4.6%. Likewise, when extracting with a mixture of equal parts of furfural and parachlorphenol, the residual carbon content ranged from 5 2.6 to 4.7%, not greatly different than with the furfural absent.

With 50% furfural, it would be normal to expect the residual carbon content of the raffinate to lie midway between the values obtained with 10 the individual solvents alone when extracting to produce the same yield. Contrary to expectation, however, the residual carbon content of the raffinate produced with the mixed solvent 15 is almost as low as with parachlorphenol alone.

Table II shows the relationship between viscosity index and yield of raffinate when extracting with the three solvent liquids.

TABLE II  
20 Viscosity index of raffinate (Dean & Davis)

| 25 | Raffinate, percent by volume | Solvent         |                        |                                      |
|----|------------------------------|-----------------|------------------------|--------------------------------------|
|    |                              | Furfural<br>(1) | Parachlorphenol<br>(2) | Furfural plus parachlorphenol<br>(3) |
| 55 | 55                           | 90+             | 88                     | 90+                                  |
| 65 | 65                           | 90+             | 78                     | 90+                                  |
| 70 | 70                           | 90+             | 76                     | 88                                   |
| 80 | 80                           | 78.5            | 66                     | 76.5                                 |
| 85 | 85                           | 73.5            | 63.5                   | 72.5                                 |

Table II shows that, when extracting with furfural alone to produce a raffinate amounting 35 to 55% by volume of the residuum, such raffinate will have a viscosity index of above 90, and when extracting to produce the same volume of raffinate with parachlorphenol the viscosity index is 30 88. However, when extracting with a mixture of equal parts of furfural and parachlorphenol, the viscosity index is still above 90. The same effect is observed when extracting to produce successively higher yields of raffinate, except that with higher yields the reduction in 45 viscosity index of the raffinates obtained with the parachlorphenol alone is quite marked.

For example, when extracting to obtain a raffinate amounting to 70% by volume of the residuum, the raffinate so obtained with furfural 50 alone has a viscosity index above 90, while that obtained with parachlorphenol alone has a viscosity index of only 76. However, the raffinate obtained when employing a mixture of furfural and parachlorphenol is 88, or very nearly the 55 same as when using the furfural alone. This shows the advantage of employing a mixture of furfural and parachlorphenol from the standpoint of obtaining a maximum yield of high viscosity index oil.

60 As already stated above, the furfural acts as an anti-solvent, offsetting the solvent action of the parachlorphenol for the more paraffinic constituents of the oil.

Thus, as indicated by the foregoing tables, it 65 is possible to employ the solvent mixture of my invention so as to obtain from residual lubricating oil a raffinate oil of relatively low residual carbon content without sacrificing the yield of high viscosity index oil.

70 Thus, from a residuum of the above type, it is possible to produce a raffinate oil amounting to 55 to 70% of the residuum, and having a viscosity index of around 90 and above with a residual carbon content of around 2 to 4%.

75 In practicing my invention, it is contemplated

that the extraction may be carried out in either stage or continuous countercurrent contact. It is also contemplated that the extraction may be carried out in the presence of a diluent solvent, such as propane or other somewhat similar low-boiling petroleum hydrocarbon. 5

Where a continuous countercurrent operation is used, it is advantageous to employ a packed tower. The residuum to be treated is introduced to the lower portion of such tower, while the solvent mixture is introduced to the upper portion. The solvent and oil flow countercurrently to each other through the tower, and form extract and raffinate phases which are removed from the bottom and top of the tower, respectively. 15

The extract phase contains the low viscosity index constituents, residual carbon-forming constituents, and dark-colored bodies dissolved in the bulk of the solvent liquid, while the raffinate phase comprises the high viscosity index constituents substantially free from residual carbon-forming and dark-colored bodies. 20

Where a diluent solvent is employed, it may be 25 advantageous to introduce the residuum to a middle point of the tower while introducing the diluent to the lower portion thereof. In such a case, the solvent mixture is introduced to the upper portion of the tower. In any case, the mixture of oil and solvent is ultimately separated 30 into extract and raffinate phases, as stated above.

As a further modification of the invention, the residual oil may be subjected to a preliminary de-asphalting treatment prior to extracting with the mixture of furfural and chlorphenol. For example, the residuum may be diluted with propane in the proportion of about four or five parts of propane to one part of residuum, and the diluted mixture subjected to settling at a temperature of around 120° F. in order to precipitate the hard 35 asphaltic constituents. The precipitated constituents are removed, and the dilute solution of residuum in propane, containing soft or resinous asphaltic constituents, is then subjected to extraction with the mixture of furfural and chlorphenol at a temperature of around 120° F. or 40 thereabouts, or at a different temperature if desired, in order to remove low viscosity index constituents and the remaining asphaltic and dark-colored constituents. 45

While a mixture containing equal parts of parachlorphenol and furfural has been mentioned above, it is contemplated that the composition of the solvent may be varied. For example, it 50 may be advantageous to employ a solvent mixture containing 25% to 75% by weight of furfural. The ratio of solvent mixture to oil employed in carrying out the extraction can be chosen to produce the desired degree of refining action. Usually, from one to four parts of solvent mixture to 60 one part of oil by volume are employed.

Obviously, many modifications and variations of the invention, as hereinbefore set forth, may be made without departing from the spirit and scope thereof, and therefore only such limitations 65 should be imposed as are indicated in the appended claim.

I claim:

In the solvent refining of residual lubricating oil containing hard and soft asphalt, dark-colored 70 constituents, and oil of low and high viscosity index and which involves extraction of the oil with a primary selective solvent consisting of furfural, the method which comprises diluting the oil with a low boiling petroleum fraction com- 75

prising propane sufficient in amount to precipitate hard asphaltic constituents, removing the precipitated hard asphaltic constituents while retaining soft asphaltic constituents in the mixture, extracting the partially deasphaltered mixture with furfural in the presence of a secondary selective solvent consisting of the isomers of chlorophenol, including ortho and para, and containing around

60 to 70% of the para isomer, forming an extract phase comprising low viscosity index, asphaltic and dark-colored constituents dissolved in the bulk of the solvent, and a raffinate phase comprising high viscosity index oil mixed with some of the solvent, and separating the two phases.

LEON W. COOK.